# EUROPEAN PATENT SPECIFICATION

(11) **EP 1 873 215 B1**
(45) Date of publication and mention of the grant of the patent: **26.05.2010**
(21) Application number: 07290694.4
(22) Date of filing: 05.06.2007
(51) Int. Cl.: C09D 11/00, B41J 2/17

(54) **Filling liquid for ink supply system**
Füllflüssigkeit für einen Tintenzufuhrsystem
Liquide de remplissage pour système de distribution d'encre

(30) Priority: 14.06.2006 JP 2006164208
(43) Date of publication of application: 02.01.2008
(73) Proprietor: Mimaki Engineering Co., Ltd., Tomi-shi, Nagano 389-0512 (JP)
(72) Inventor: Hijikata, Yasuyuki, Tomi-City, Nagano (JP); Shimada, Nami, Tomi-City, Nagano (JP); Namiki, Takashi, Tomi-City, Nagano (JP); Tabayashi, Isao, Tomi-City, Nagano (JP); Mitsui, Takayuki, Tomi-City, Nagano (JP)
(74) Representative: Uchida, Kenji

(56) References cited:
- EP-A1- 1 074 589
- EP-A1- 1 473 338
- US-A1- 2004 035 322
- US-A1- 2005 018 023
- DATABASE WPI Week 200575 Derwent Publications Ltd., London, GB; AN 2005-729231 XP002451802 & JP 2005 288728 A (RISO CHEM IND CO LTD) 20 October 2005 (2005-10-20)

## Description

### TECHNICAL FIELD

The present invention relates to a filling which is incorporated into an ink supply system at the time of storing or conveying an inkjet device or inkjet head utilizing a solvent base ink, and belongs to a technical field of filling liquid for an ink supply system which avoids blockage of a nozzle possessed by the inkjet head and which prevents poor discharge brought about with finally substituting solvent base ink.

### BACKGROUND ART

Since it is required for a lot of time and lobar to adjust discharge of solvent base ink at a place where a printer is set, it is desirable to perform discharge adjustment in advance at the time of shipping the printer. In this case, when conveying the inkjet head with the solvent base ink filling with the solvent base ink, the blockage of the nozzle accompanying the solidification of the solvent base ink will often occur. In order to avoid the blockage, a method can be considered which detracts the solvent base ink and washes the nozzle with a cleaning liquid. However, this method cannot perfectly wash the nozzle and has a problem concerning the solidification of the residual ink.

As a filling liquid for an inkjet head, various fillings have been known, and for example, a filling comprising a non-volatile organic solvent, especially water-soluble organic solvent and a filling containing water and 1,2-hexane diol have been suggested (Japanese Patent Laid-Open No. 09-327934, and Japanese Patent Laid-Open No. 2004-243543). These fillings are filling substantially used for a water base ink. A filling for inkjet head comprising non-water solvent containing alcoholic solvent having a boiling point of from 150 to 350°C aimed at an oil base ink has been suggested (Japanese Patent Laid-Open No. 2005-288728), but it is difficult to avoid the aggregation of pigments in the ink stored over a prolonged period of time and to avoid adherend to nozzle head. An inkjet recording device has been suggested which fill a head with a UV ink from which a photo-curing initiator is removed (Japanese Patent Laid-Open No. 2005-1302), but this technique is for a filling for a UV ink and, thus, is not suitable for an inkjet recording device utilizing a solvent base ink.

As how to cope effectively with the problems described above, a method can be mentioned, which fills an ink supply system with a filling based on an organic solvent having a high boiling point and resembling the component of the solvent of the solvent base ink and which stores and conveys the head. However, this method also has problems associated with instable flying of the ink particles and with non-discharge of ink due to adherend around the nozzle (one of blockage of nozzle).

The present invention has been made in light of the problems mentioned above, and an object of the present invention is to provide a filling liquid for an ink supply system with which an inkjet device or an inkjet head is filled at the time of its storage or conveying, and which can avoid the blockage of the nozzle of the inkjet head and which can prevent poor discharge brought about with the finally substituting solvent base ink.

### SUMMARY OF THE INVENTION

The object described above and other objects of the present invention can be attained by the following constitutions as defined in the claims.
Specifically, according to the present invention there is provided a filling liquid for an ink supply system with which an ink supply system is filled instead of an ink, which contains an organic solvent having a boiling point of at least 150°C and fluorine series surfactant.
In the filling liquid for an ink supply system according to the present invention, at least one of the organic solvent component in the solvent base ink and the organic solvent component in the filling for the ink supply system is an organic solvent having a glycol ether group in the chemical structure thereof.
In the filling liquid for an ink supply system according to the present invention, a part of the organic solvent in the filling liquid for an ink supply system may be an organic amine.
In the filling liquid for an ink supply system according to the present invention, the fluorine series surfactant is preferably a nonionic type or anion type.
In the filling liquid for an ink supply system according to the present invention, the contents of the fluorine series surfactant is preferably from 10 to 10000 ppm.
In the filling liquid for an ink supply system according to the present invention, the surface tension of the filling liquid for an ink supply system is preferably from 15 to 26 mN/m.

According to the present invention a filling liquid for an ink supply system with which an inkjet device or an inkjet head is filled utilizing an solvent base ink at the time of its storage or conveying, and which can avoid the blockage of the nozzle of the inkjet head and which can prevent poor discharge brought about with the finally substituting solvent base ink.

### BRIEF DESCRIPTION OF THE DRAWINGS

FIG. 1 shows a relation among the amount of the fluorine type surfactant added in the filling liquid for an ink supply system, a viscosity and a surface tension.

### BEST MODE FOR CARRYING OUT THE INVENTION

The present invention will now be described in detail. In an inkjet device or an inkjet head utilizing a solvent base ink as in the present invention, it has been known that a filling with which an ink supply system is filled instead of the solvent base ink (the filling liquid for an ink supply system) is generally selected from organic solvent having a high boiling point and good compatibility with the solvent base ink, and the organic solvent preferably has a boiling point of not less than 200°C. However, in some cases, after the filling liquid for an ink supply system is substituted with the solvent base ink, the direction of flying the ink particle become instable and, in the worst case, foreign substances are often adhered within or around the nozzle. In particular, even in the case where once the ink supply system is filled with the solvent base ink, the discharge adjustment of the ink head is performed, then the ink supply system is thoroughly washed, and the filling liquid for an ink supply system is incorporated within the ink supply system, this problem occurs significantly, when the washing of the ink supply system is not performed in a perfect manner and the filling is substituted with the solvent base ink after stored or conveyed over a prolonged period of time, and the ink is again discharged.

We have deduced that the caused thereof are as follows: (1) When the conventionally utilized fill for ink supply system is in contact with the solvent base ink, the ink components become instable, adhering them onto the interior of the nozzle of the inkjet head. This results in the generation of cavitation taking the portion to which the ink components are adhered as a core, and in change in the direction of flying the ink particle and the non-discharge of the ink due to the adhrend around the nozzle. (2) When the washing liquid comprising a solvent highly compatible with the solvent base ink (including the organic solvent for the filling according to the present invention, which will be described later on) as a main component is used to wash the ink supply system, particularly the nozzle, the pigments or resins which are components of the ink are adhered onto the interior and/or edge surface of the nozzle due to so-called solvent shock, easily leading to the phenomenon similar to those described under (1). These phenomenons are said to be blockage of the nozzle in a wide sense.

The blockage of the nozzle in the wide sense occurs remarkable, when the ink is a pigment ink.

We have investigated the composition of the filling liquid for an ink supply system in which the ink components becomes instable to minimum when the filling liquid for an ink supply system or the washing liquid is in contact with the solvent base ink, particularly pigment dispersion type ink, to prevent the adhesion of the components onto the interior of the nozzle, and even if the ink components are adhered onto the nozzle, the extent thereof can reduce to minimum. Specifically, when we have tried application of a filling liquid for an ink supply system based on an organic solvent having a high boiling point and resembling a solvent component of the solvent base ink to which various additives (for example, a pigment dispersant, an antioxidant, an amine series stabilizer and the like) and a general surfactant are added, no remarkable improvement has not been obtained. Under such a circumference, we have discovered that a filling liquid for an ink supply system containing an organic solvent having a boiling point of not less than 150°C, preferably at least 200°C and fluorine series surfactant has an excellent effect. Different from the general surfactant, it can be considered that due to excellent wetting property, disperibility with the pigment and washing property possessed by the fluorine surfactant, the prevention of aggregation of the ink remaining within the ink supply system and the pigments contained in the ink during the course of substituting the filling liquid for an ink supply system with the solvent base ink and the prevention of adhesion onto the interior of the nozzle are imparted, and the joint use of the organic solvent having a high boiling point makes the interior of the nozzle always wet even after stored over a long period of time.

The organic solvent component contained in solvent base ink and the organic solvent component contained in the filling liquid for an ink supply system according to the present invention are preferably compatible with each other. More preferably, they are organic solvent components each having resembling chemical structure.

The organic solvent component contained in the solvent base ink is an organic solvent having a glycol ether group within the chemical structure thereof such as glycol ether, and glycol ether acetate. The filling liquid for an ink supply system according to the present invention contains an organic solvent also having a glycol ether group within the chemical structure thereof.

Examples of an organic solvent having a boiling point of not less than 150°C, preferably at least 200°, making up the filling liquid for an ink supply system, include, but are not restricted to : alcohols such as n-hexyl alcohol (boiling point153°C), isoheptyl alcohol (boiling point 168°C), 2-ethylhexyl alcohol (boiling point 184°C), n-octyl alcohol (boiling point 194°C), 3-methyl-3-methoxy butanol (boiling point 174°C), 3-methoxybutanol (boiling point 160°C); hydrocarbons such as terpin oil (boiling point 155°C), limonene (boiling point 178°C), industrial volatile oil (boiling point 150°C or more), tetrahydronaphthalene (boiling point 207°C), and decahydronaphthalene (boiling point 190°C); glycols such as ethylene glycol (boiling point 197°C), diethylene glycol (boiling point 244°C), thiodiethylene glycol (boiling point 168°C), triethylene glycol (boiling point 287°C), proplylene glycol (boiling point 187°C), dipropylene glycol (boiling point 232°) and tripropylene glycol (boiling point 265°C); glycol ether esters such as ethylene glycol monoethyl ether acetate (boiling point 156°C), ethylene glycol monobutyl ether acetate boiling point 191°C), diethylene glycol monoethyl ether acetate (boiling point 219°C), diethylene glycol monobutyl ether acetate (boiling point 238-248°C), dipropylene glycol monomethyl ether acetate (boiling point 200°C), and borate of triethylene glycol monomethyl ether (boiling point 275°C); glycol ethers such as ethylene glycol monohexyl ether (boiling point 208°C), ethylene glycol 2-ethylhexyl (boiling point 225°C), ethylene glycol phenyl ether (boiling point 245°C), proplylene glycol monoethyl ether (boiling point 158°C), propylene glycol propyl ether (boiling point 150°C), propylene glycol monobutyl ether (boiling point 170°C), diethylene glycol monomethyl ether (boiling point 194°C), diethylene glycol dimethyl ether (boiling point 162°C), diethylene glycol monoethyl ether (boiling point 203°C), diethylene glycol diethyl ether (boiling point 189°C), diethylene glycol monobutyl ether (boiling point 230°C), diethylene glycol hexyl ether (boiling point 260°C), diethylene glycol 2-ethylhexyl ether (boiling point 270°C), dipropylene glycol monomethyl ether (boiling point 188°C), dipropylene glycol monoethyl ether (boiling point 198°C), dipropylene glycol monobutyl ether (boiling point 215°C), dipropylene glycol propyl ether (boiling point 210°C), triethylene glycol monomethyl ether (boiling point 249°C), triethylene glycol monoethyl ether (boiling point 256°C), triethylene glycol monobutyl ether (boiling point 271°C), tripropylene glycol monomethyl ether (boiling point 243°C), triethylene glycol dimethyl ether (boiling point 216°C), and tetraethylene glycol dimethyl ether (boiling point 275°C); esters such as 2,2,4-trimethyl-1,3-pentadiol monoisobutylate (boiling point 253°C), triethylene glycol di (2-ethyl butylate) (boiling point 181°C), propylene carbonate (boiling point 242°C), ethyl lactate (boiling point 155°C), butyl lactate (boiling point 187°C), methyl acetoacetate (boiling point 172°C), ethyl acetoacetate (boiling point 181°C), dibasic esters DBE(boiling point 205°C), and 3-methyl-3-methoxybutyl acetate (boiling point 188°C); ketones such as 2-heptanone (boiling point 151°C), diisobutyl ketone (boiling point 170°C), isophorone (boiling point 215°C), diacetone alcohol (boiling point 168°C), acetophenone (boiling point 202°C), cyclohexanone (boiling point 155°C), γ-butyrolactone (boiling point 204°C), and 2-(1-cyclohexycenyl)cyclohexanone (boiling point 168°C); alcohol amines such as triethanol amine (boiling point 335°C), N-methyldiethanol amine (boiling point 247°C), N,N-diethylethanol amine (boiling point 163°C), and N, N-dibutylethanol amine (boiling point 230°C); organic amines such as tri-n-butyl amine (boiling point 217°C); and pyrolidones such as N-methyl-2-pyrolidone (boiling point 204°C). The organic solvents just mentioned are not restricted to the composition of the solvent base ink as long as they are good compatible with the solvent ink. The organic solvents having a high boiling point generally have high viscosity and, thus, they may be combined with an organic solvent having a low boiling point as a diluent.

Since the solvent base ink is a glycol ether having a glycol ether group in the chemical structure thereof and the filling liquid for an ink supply system is a glycol ether having a glycol ether group in the chemical structure thereof, due to its good compatibility, when being combined with the filling liquid for an ink supply system, the filling liquid for an ink supply system according to the present invention exhibits excellent performance, and even if the filling liquid for an ink supply system according to the present invention is substituted with the solvent base ink after being stored and conveyed over a prolonged period of time, change in the direction of flying the ink particle and the non-discharge of the ink based on the blockage in a wide sense as described above never occur.

Amongst the organic solvents described above, the organic amines have a merit of exhibiting prevention of corrosion, if they are added in a small amount, when ink head material easily undergoes corrosion with a trace amount of acid component generated according to the oxidation of the glycol ether type organic solvent or with chlorine ion contaminated in a trace amount

The fluorine series surfactant which is an essential component for the filling liquid for an ink supply system, may be any of anion types, nonion types and cation types, and exemplified compounds include, but are not restricted to, low molecular compounds having fluorine such as perfluoroalkyl sulfonates, ethylene oxide adducts of perfluroroalkyls, trimethyl ammonium salts of perfluoroalkyls, perfluoroalkyl aminosulfonates, oligomers having a perfluoroalkyl group and a lipophilic group in the chemical structure thereof, oligomers having a perfluoroalkyl group and an hydrophilic group in the chemical structure thereof, urethanes having a perfluoroalkyl group and a lipophilic group in the chemical structure thereof, perfluoroalyl phosphates, perfluoroalyl carboxylates, perfluoroalkyl amine compounds, quaternary ammonium salts of perfluoroalyls, perfluoroalkyl betains, non-soluble perfluoroalkyl compounds, and fluorine silicone oils

Examples of commercially available fluorine series surfactants includes, but are not restricted to, MRGAFAX® F110, MRGAFAX® F-114, MRGAFAX® F-120, MRGAFAX® F-142D, MRGAFAX® F-144D, MRGAFAX® F-172D, MRGAFAX® F-173, MRGAFAX® F-177, MRGAFAX®F-183, MRGAFAX®F-191, MRGAFAX® F-445, MRGAFAX® F-470, MRGAFAX® F-471, MRGAFAX® F-479, MRGAFAX® F-493, and MRGAFAX® F-494 (available from DAINIPPON INK AND CHEMICALS, INCORPORATED); Flourad FC-93, Flourad FC-95, Flourad FC-129, Flourad FC-170, Flourad FC-171, Flourad FC-430, Flourad FC-431, Flourad EF301, Flourad EF303, and Flourad EF352 (available from Sumitomo 3M Co., Ltd.); F-TOP EF-122B, and F-TOP EF802 (available from Shin Akita Chemicals Co., Ltd.); Asahi Guard AG710, Surflron S-382, Surflron S-382, Surflron SC-101, Surflron SC-102, Surflron SC-103, Surflron SC-104, Surflron SC-105, and Surflron SC-102 (available from Asahi Glass Corporation); BM-1000, and BM-1100 (available from Yosho Co., Ltd.) ; and NBX-15 (available fro NEOS Co., Ltd). They can be used jointly. Amongst them, MRGAFAX® F-114 (anionic type), MRGAFAX® F-445 (nonionic type), MRGAFAX® F-470 (nonionic type), MRGAFAX® F-471 (nonionic type), MRGAFAX® F-479 (nonionic type), MRGAFAX® F-493 (nonionic type), and MRGAFAX® F-494 (anionic type) are preferable in terms of excellent washing ability and pigment dispersibility. In particular, nonionic type fluorine series surfactants are in a liquid form in a single state and, thus, even if the organic solvent component is volatilized, they exhibit a function of preventing the nozzle from being dried to be solid state.

The content of the fluorine series surfactant in the filling liquid for an ink supply system according to the present invention is not specifically restricted, but if it is too small, the effect exhibited by filling the ink supply system is small, and conversely if it is too large, viscosity of the filling liquid for an ink supply system is increased and the viscosity is increased according to volatilization of the organic components in the filling liquid for an ink supply system. Consequently, the content of the fluorine series surfactant is preferably from 10 to 10000 ppm, and more preferably from 10 to 5000 ppm.

The surface tension of the filling liquid for an ink supply system prepared after adding the fluorine series surfactant described above is preferably in the range of from 15 to 26 mN/m.

In the filling liquid for an ink supply system according to the present invention, as occasion demands, organic solvent having a boiling point of not more than 150°C may be jointly used (mixed). If the ink is a pigment dispersion type solvent base ink, a pigment dispersant, other antioxidant, various stabilizers, and other surfactant may be jointly used (mixed).

The filling liquid for an ink supply system according to the present invention exhibits excellent performance as the filling liquid for an ink supply system unless the solvent base ink and the filling liquid for an ink supply system are compatible with each other. Consequently, the filling liquid for an ink supply system according to the present invention can be applied to various inkjet systems utilizing various solvent base inks.

It is also possible that the ink supply system is washed with a washing liquid having a low viscosity and excellent compatibility with the ink before it is filled with the filling liquid for an ink supply system according to the present invention.

### EXAMPLES

The present invention will be described in more detail by referring to working examples. It is however should be noted that the present invention is not restricted to the working examples.

### EXAMPLE 1

### (PREPARATION)

First, as the filling liquid for an ink supply system according to the present invention, fillings for an ink supply were prepared, comprising an organic solvent having a glycol ether group in the molecule thereof (tetraethylene glycol dimethyl ether (boiling point 275°C) in an amount of not lower than 50 wt% to which an oligomer having a perfluoroalkyl group, a hydrophilic group, and a lipophilic group in the chemical structure thereof (nonionic type (MEGAFAX® F-494 (available from DAINIPPON INK AND CHEMICALS, INCORPORATED) in an amount of 10 ppm, 100 ppm, 1000 ppm, and 10000 ppm, respectively as a fluorine series surfactant.

As the solvent base ink, which was used, was a pigment dispersion type solvent base ink containing 75 wt% of ethylene glycol methylethyl ether. When the filling liquid for an ink supply system according to the present invention prepared as described above was mixed with the solvent base ink used in Example 1 in a proportion of 1:1, they were compatible with each other, confirming that the filling liquid for an ink supply system in Example 1 had good compatibility.

### (TEST UPON REAL MACHINE)

A new head was fitted to an inkjet device utilizing a solvent base ink (solvent base ink type inkjet device), and an ink supply system (ink supply tube, and inkjet head (nozzle)) was washed with a washing liquid (diethylene glyxol dimethyl ether). Thereafter, the ink supply system was filled with a solvent base ink, and the discharge adjustment of the inkjet head was performed. Subsequently, the solvent base ink was detracted, and the ink supply system was washed with the washing liquid for a solvent base ink. Subsequently, the ink supply system was filled with the filling liquid for an ink supply system according to the present invention, prepared as described above, and the system was stored at 60°C for seven days and at -20°C for 7 days, which elapsed a time under the situations considered to be long term storage and conveying.

Thereafter, the filling liquid for an ink supply system was exhausted out of the ink supply system, and the ink supply system was left standing at a normal temperature for 30 minutes.

Subsequently, the ink supply system was again filled with the solvent base ink, and test drawing and test printing were conducted.

### (EVALUATION)

(1) It has been confirmed that there was substantially no coming off (non-discharge of ink) and no curve in the tested drawing.
(2) Furthermore, it has been confirmed that there was no strip generated due to instable flying direction of ink particles by a solid printing (phenomenon that the strip visibly appears).
(3) In addition, when the nozzle side (discharge hole) of the inkjet head was microscopically observed it has been confirmed that there was no or little adhesion onto the side of the nozzle (no one of nozzle blockage).

### COMPARATIVE EXAMPLE 1

Example 1 was repeated except that a filling liquid for an ink supply system adding no fluorine series surfactant was used in preparation of Example 1.

As a result, it has been confirmed the non-discharge of ink was remarkable and strips occurred significantly. Also, there was adhesion on the nozzle side (within and around the discharge hole), the head was required to be replaced.

The filling liquids for ink supply system used in Example 1 and Comparative Example 1 were tested for viscosity and surface tension (at a normal temperature of 25°C. The results are shown in FIG. 1 (Change in Physical Properties). It has been understood from FIG. 1 that in comparison with the surface tension of Comparative Example, which was 33.5 mN/M, in which no fluorine series surfactant was added, the surface tension was decreased in Example 1 in which the fluorine series surfactant was added, and particularly, in the case of adding the fluorine series surfactant was added in an amount of approximately 1000 ppm, the surface tension was much more decreased, indicating excellent wetting property. From viewpoint of suppressing the increasing of the viscosity, it has been found that the amount of the fluorine series surfactant was preferably not more than approximately 1000 ppm.

### EXAMPLE 2

Example 1 was repeated except that tri-n-butyl amine (boiling point 217°C) was added to the organic solvent used in Example 1 in an amount of 0.1 wt%.

This gave similar results.

### EXAMPLE 3

Example 1 was repeated except that a fluorine series surfactant different from that of Example 1 (fluorine series surfactant containing perfluorobutyl sulfonate: MEGAFACE® F-114 (Anionic type), available from DAINIPPON INK AND CHEMICALS, INCORPORATED) was used as the fluorine series surfactant in the filling liquid for an ink supply system.

This gave similar results.

### EXAMPLE 4

Example 1 was repeated except that a filling liquid for an ink supply system (viscosity: 4.00 mPa.s, surface tension : 25.9 mN/m) containing 1000 ppm of MEGAFACE® F-479 and 1000 ppm of MEGAFACE® F-479 (both available from DAINIPPON INK AND CHEMICALS, INCORPORATED) was used as the fluorine series surfactant instead of single use of MEGAFACE® F-479.111

This gave similar results.

Particularly, no nozzle abnormality could be found after high temperature storage for 7 days at 60°C.

### EXAMPLE 5

Example 1 was repeated except that an organic solvent different from that of Example 2 (propylene carbonate; boiling point 242°C) was used as the organic solvent in the filling liquid for an ink supply system.

This gave similar results.

### EXAMPLE 6

Example 1 was repeated except that a pigment dispersant type solvent base ink (an organic solvent comprising a mixture of cyclohexanone, dipropylene glycol dimethyl ether, dipropylene glycol dimethyl ether, and dipropylene glycol methylethyl ether acetate) different from the solvent base ink used in Example 1 was used.

This gave similar results.

As described above, the filling liquid for an ink supply system according to the present invention is effectively used in a method for storing and conveying a solvent type inkjet device and a solvent type inkjet head in which the ink supply system is once filled with a solvent base ink, for example, the discharge adjustment of the ink head is performed, the solvent is detracted and the ink supply system is well washed, after which the ink supply system is filled with the filling liquid for an ink supply system, the storage or conveying is performed in this state, then the filling liquid for an ink supply system is exhausted, and then the ink supply system is again filled with the solvent base ink.

In the above-mentioned fact, it is useful as means for avoiding the generation of a phenomenon that a pigment or resin is adhered onto the interior of the nozzle or the edge surface of the nozzle due to so-called solvent shock to wash the ink supply system, particularly, the nozzle, with a washing liquid comprising an organic solvent having a low density and having a high compatibility with the solvent ink (including the organic solvent for the filling liquid for an ink supply system according to the present invention) at the time of detracting the solvent base ink and washing the ink supply system.

The filling liquid for an ink supply system according to the present invention can also be used for the application that before the ink supply system in the solvent type inkjet device or the solvent type inkjet head is first filled with the solvent base ink, the solvent type inkjet device or the solvent type inkjet head is stored or conveyed in the state where the ink supply system is filled with the filling liquid according to the present invention.

## Claims

1. A set comprising:
a solvent ink comprising an organic solvent components; and
a filling liquid for an ink supply system of an inkjet apparatus or a an inkjet head using the solvent ink, said filling liquid being used to fill an ink supply system instead of said solvent ink, said filling liquid comprising at least an organic solvent having a boiling point of 150°C or more, wherein:
both said organic solvent components in the solvent ink and said organic solvent components in the filling liquid comprise at least one glycol ether group in the chemical structure thereof; and
said filling liquid further comprises fluorine series surfactant.

2. The set according to claim 1, wherein the contained amount of said glycol ether group in said filling liquid is not lower than 50%wt.

3. The set according to claim 1 or 2, wherein a part of the organic solvent components in the filling liquid is organic amine.

4. The set according to any one of claims 1 through 3, wherein said fluorine series surfactant is of a nonionic type or of an anion type.

5. The set according to any one of claims 1 through 4, wherein the contained amount of the fluorine series surfactant in said filling liquid is in a range from 10 to 10,000 ppm.

6. The set according to any one of claims 1 through 5, wherein the surface tension of the filling liquid is in a range from 15 to 26 mN/m.

7. A use of a solvent ink and a filling liquid according to any one of claims I to 6, for storing and conveying an ink supply system of an inkjet apparatus or a an inkjet head, said filling liquid being used to fill an ink supply system instead of said solvent ink.

8. A process for storing and conveying an ink supply system of an inkjet apparatus or an inkjet head using the solvent ink, wherein the process comprises steps of:
filling said ink supply system with a solvent ink according to claim 1;
discharge adjustment of said ink head;
detracting the solvent and washing said ink supply system; and
the ink supply system is filled with the filling liquid according to any one of claims 1 through 6.

9. The process for storing and conveying the ink supply system of the inkjet apparatus or an inkjet head using the solvent ink according to claim 8, wherein the process further comprises steps of:
exhausting said filling liquid in the ink supply system; and
filling the ink supply system with the solvent base ink.

## Patentansprüche

1. Set, umfassend:
eine Lösungsmitteltinte, umfassend organische Lösungsmittelkomponenten;
und
eine Füllflüssigkeit für ein Tintenzufuhrsystem einer Tintenstrahlvorrichtung oder eines Tintenstrahlkopfes, welche die Lösungsmitteltinte verwenden, wobei die Füllflüssigkeit zum Füllen eines Tintenzufuhrsystems, anstatt der Lösungsmitteltinte, verwendet wird, wobei die Füllflüssigkeit mindestens ein organisches Lösungsmittel mit einem Siedepunkt von 150°C oder mehr umfasst,
wobei:
sowohl die organischen Lösungsmittelkomponenten in der Lösungsmitteltinte als auch die organischen Lösungsmittelkomponenten in der Füllflüssigkeit mindestens eine Glykolether-Gruppe in deren chemischer Struktur umfassen; und
wobei die Füllflüssigkeit weiter ein grenzflächenaktives Mittel der Fluorserie umfasst.

2. Set nach Anspruch 1, wobei die enthaltene Menge der Glykolether-Gruppe in der Füllflüssigkeit nicht weniger als 50 Gewichtsprozent beträgt.

3. Set nach Anspruch 1 oder 2, wobei ein Teil der organischen Lösungsmittelkomponenten in der Füllflüssigkeit organisches Amin ist.

4. Set nach einem der Ansprüche 1 bis 3, wobei das grenzflächenaktive Mittel der Fluorserie vom nichtionischen Typ oder vom anionischen Typ ist.

5. Set nach einem der Ansprüche 1 bis 4, wobei die enthaltene Menge des grenzflächenaktiven Mittels der Fluorserie in der Füllflüssigkeit in einem Bereich von 10 bis 10.000 ppm liegt.

6. Set nach einem der Ansprüche 1 bis 5, wobei die Oberflächenspannung der Füllflüssigkeit in einem Bereich von 15 bis 26 mN/m liegt.

7. Verwendung einer Lösungsmitteltinte und einer Füllflüssigkeit nach einem der Ansprüche 1 bis 6 für das Lagern und das Befördern eines Tintenzufuhrsystems einer Tintenstrahlvorrichtung oder eines Tintenstrahlkopfes, wobei die Füllflüssigkeit zum Füllen eines Tintenzufuhrsystems, anstatt der Lösungsmitteltinte, verwendet wird.

8. Verfahren zur Lagerung und Beförderung eines Tintenzufuhrsystems einer Tintenstrahlvorrichtung oder eines Tintenstrahlkopfes, welche die Lösungsmitteltinte verwenden, wobei das Verfahren die Schritte:
des Befüllens des Tintenzufuhrsystems mit einer Lösungsmitteltinte nach Anspruch 1;
des Einstellens des Ausstoßes des Tintenkopfes;
des Entfernens des Lösungsmittels und des Waschens des Tintenzufuhrsystems; und
des Befüllens des Tintenzufuhrsystems mit der Füllflüssigkeit nach einem der Ansprüche 1 bis 6
umfasst.

9. Verfahren zur Lagerung und Beförderung eines Tintenzufuhrsystems einer Tintenstrahlvorrichtung oder eines Tintenstrahlkopfes, welche die Lösungsmitteltinte verwenden, nach Anspruch 8, wobei das Verfahren weiter die Schritte:
des Entfernens der Füllflüssigkeit in dem Tintenzufuhrsystem; und
des Befüllens des Tintenzufuhrsystems mit der Lösungsmittelbasistinte umfasst.

## Revendications

1. Ensemble comprenant :
une encre à base de solvant comprenant des composants formant solvant organique ; et
un liquide de remplissage pour un circuit d'alimentation en encre d'un dispositif à jet d'encre ou d'une tête à jet d'encre utilisant l'encre à base de solvant, ledit liquide de remplissage étant utilisé afin de remplir un circuit d'alimentation en encre au lieu de ladite encre à base de solvant, ledit liquide de remplissage comprenant au moins un solvant organique présentant un point d'ébullition supérieur ou égal à 150°C, dans lequel :
à la fois lesdits composants formant solvant organique dans l'encre à base de solvant et lesdits composants formant solvant organique dans le liquide de remplissage comprennent au moins un groupe éther glycol dans leur structure chimique ; et
ledit liquide de remplissage comprend, en outre, un surfactant à base de fluor.

2. Ensemble selon la revendication 1, dans lequel la teneur dudit groupe éther glycol dans ledit liquide de remplissage n'est pas inférieure à 50 % en poids.

3. Ensemble selon la revendication 1 ou 2, dans lequel une partie des composants formant solvant organique dans le liquide de remplissage est une amine organique.

4. Ensemble selon l'une quelconque des revendications 1 à 3, dans lequel ledit surfactant à base de fluor est d'un type non ionique ou d'un type anionique.

5. Ensemble selon l'une quelconque des revendications 1 à 4, dans lequel la quantité de surfactant à base de fluor contenue dans le liquide de remplissage est comprise dans une plage de 10 à 10 000 ppm.

6. Ensemble selon l'une quelconque des revendications 1 à 5, dans lequel la tension superficielle du liquide de remplissage est comprise dans une plage de 15 à 26 mN/m.

7. Utilisation d'une encre à base de solvant et d'un liquide de remplissage selon l'une quelconque des revendications 1 à 6, afin de stocker et de transporter un circuit d'alimentation en encre d'un dispositif à jet d'encre ou d'une tête à jet d'encre, ledit liquide de remplissage étant utilisé afin de remplir un circuit d'alimentation en encre plutôt que ladite encre à base de solvant.

8. Procédé de stockage et de transport d'un circuit d'alimentation en encre d'un dispositif à jet d'encre ou d'une tête à jet d'encre utilisant l'encre à base de solvant, dans lequel le procédé comprend les étapes de :
remplissage dudit circuit d'alimentation en encre avec une encre à base de solvant selon la revendication 1 ;
réglage de débit de sortie de ladite tête à jet d'encre ;
diminution du solvant et lavage dudit circuit d'alimentation en encre ; et
le circuit d'alimentation en encre est rempli du liquide de remplissage selon l'une quelconque des revendications 1 à 6.

9. Procédé de stockage et de transport du circuit d'alimentation en encre du dispositif à jet d'encre ou d'une tête à jet d'encre en utilisant l'encre à base de solvant selon la revendication 8, dans lequel le procédé comprend, en outre, les étapes de :
évacuation dudit liquide de remplissage dans le circuit d'alimentation en encre ; et
remplissage du circuit d'alimentation en encre avec l'encre à base de solvant.
